

## UNITED STATES PATENT OFFICE

2,591,570

## CUTTING OIL

Samuel Manilich, Brooklyn, and Lee L. Lambert,  
Flushing, N. Y., assignors to Socony-Vacuum  
Oil Company, Incorporated, New York, N. Y., a  
corporation of New York

No Drawing. Application April 8, 1949,  
Serial No. 86,383

13 Claims. (Cl. 252—48.4)

**1**  
The present invention relates to mineral oil compositions comprising a base oil of petroleum origin and hydroabietyl alcohol and, more particularly, to mineral oil compositions suitable for use as cutting oils and containing a mixture of hydrogenated abietyl alcohols and rosin hydrocarbons.

Dehydroabietyl alcohol, dihydroabietyl alcohol and tetrahydroabietyl alcohol together with a small proportion of esters of hydrogenated rosin and hydrocarbons are available industrially under the name "hydroabietyl alcohol." The mixture available to industry under the name hydroabietyl alcohol is composed of 13-15 per cent of a non-alcohol fraction and the balance of a mixture of hydrogenated abietyl alcohols in which about 15 per cent is dehydroabietyl alcohol, about 40 per cent is dihydroabietyl alcohol and the balance, about 45 per cent, is tetrahydroabietyl alcohol. The non-alcohol portion of hydroabietyl alcohol varies with the saponification number but will average about 3-8 per cent of the total mixture in the form of esters which can be considered as methyl esters of hydrogenated rosin and the remainder, 7-12 per cent of the total mixture, is similar to the hydrocarbon fractions occurring in hydrogenated rosin.

The physical properties and composition of the material available under the name hydroabietyl alcohol and comprising the aforesaid mixture of alcohols, esters and hydrocarbons are as follows:

|                                                               |                  |
|---------------------------------------------------------------|------------------|
| Hydroxyl value.....                                           | 5.0-5.1 per cent |
| Hydroabietyl alcohol.....                                     | 85-87 per cent   |
| Saponification number (diethyl-<br>ene glycol method).....    | 5-14             |
| Acid number.....                                              | 0.1-0.4          |
| Methoxyl value.....                                           | 0.5-1.2          |
| Unsaturation: weight per cent—<br>By hydrogen absorption..... | 0.60-0.75        |
| By bromine number.....                                        | 12-30            |
| Color (50 mm. tube) Lovibond.....                             | 0.5 amber        |
| U. S. Rosin Standard.....                                     | Z <sup>1</sup>   |
| Softening point (drop method).....                            | 33° C.           |
| Specific gravity at 20°/20° C.....                            | 1.007-1.008      |

**2**  
Refractive index at 20° C..... 1.528  
Flash point (C. O. C.)..... 185-195° C.  
Flame point (C. O. C.)..... 217-220° C.

It has long been the practice to enhance the value of mineral oil for use as a cutting lubricant by the addition of various materials such as esters to the lubricating fraction of mineral oil. Other cutting oils having as bases sulfurized mineral oil, chlorinated mineral oil or sulfurized and chlorinated mineral oil or a mixture of sulfurized mineral oil and chlorinated mineral oil in combination with a lubricating fraction of mineral oil of suitable viscosity have also been used in conjunction with additives such as esters, and stain inhibitors. The ester type of additive, particularly those made by esterifying an hydroxy aliphatic dicarboxylic acid with a monohydric aliphatic alcohol having more than 10 carbon atoms in the molecule and those made by esterifying one hydroxyl group of a low molecular weight dihydric alcohol with an aliphatic acid having more than 10 carbon atoms in the molecule and then esterifying the other hydroxyl group of the dihydric alcohol with an hydroxyl aliphatic dicarboxylic acid has been found particularly useful as an oiliness additive. It now has been discovered that vastly improved results can be produced by employing the aforescribed hydroabietyl alcohol as an oiliness agent in the formulation of cutting oils.

Before describing the novel cutting oil compositions it is believed well to identify the alcohols present in hydroabietyl alcohol and indicate the probable structure thereof. The hydroabietyl alcohol industrially available is composed of an alcohol fraction and a non-alcohol fraction. As noted hereinbefore about 3-8 per cent of the total mixture is esters which may be considered methyl esters of hydrogenated rosin and about 7-12 per cent of the total mixture is similar to the hydrocarbon fractions occurring in hydrogenated rosin. The balance is about 14-23 per cent dehydroabietyl alcohol, about 38-39 per cent dihydroabietyl alcohol and about 38-50 per cent

tetrahydroabietyl alcohol. It will be observed that the structures of both dehydroabietyl alcohol and dihydroabietyl alcohol are structures of unsaturated alcohols and that all three alcohols have the hydroxyl group attached to the nucleus through a methylene group. The hydroabietyl alcohols may be considered as related to phenanthrene. This relationship is recognized readily by consideration of the following structural formulae:



The effectiveness of "hydroabietyl alcohol," i. e., the commercially available mixture of the three hydroabietyl alcohols, hydrocarbons and methyl esters of hydrogenated rosin was compared with that of two ester type additives in a moderately sulfurized oil containing 0.9 per cent active sulfur. The blends tested comprised 99 parts by weight sulfurized pale oil having a viscosity of 150 S. U. seconds @ 100° F. and containing about 0.9 per cent active sulfur and 1 per cent of the ester type additive, 99 weight per cent sulfurized pale oil of 150 seconds SUV containing about 0.9 per cent active sulfur and 1 weight per cent of commercially available hydroabietyl alcohol, and 95 weight per cent of the sulfurized oil containing 0.9 per cent active sulfur and 5 weight per cent commercially available hydroabietyl alcohol.

The blends were subjected to three tests, viz.: tapping efficiency, Oster threading efficiency and drill life tests. These tests are performed as described hereinafter.

#### TAPPING TEST

In the measurement of tapping efficiency of an oil, a series of holes are very accurately drilled in a test metal, namely SAE 1020 hot rolled steel. These holes are subsequently tapped with a series of taps, in a drill press equipped with a table, which is free to rotate about the center, being mounted on ball bearings. A torque arm is attached to this "floating" table and this arm in turn actuates a spring scale so that the actual torque during tapping with the oil being evaluated is measured directly. The same taps used in evaluating the test oil are employed in tapping with a standard reference oil, which has arbitrarily been assigned an efficiency of 100 per cent. The average torque for the test oil is compared

to that of the standard and a relative efficiency is calculated on a percentage basis. For example:

|   |                                         |      |
|---|-----------------------------------------|------|
| 5 | Torque with standard reference oil..... | 19.3 |
|   | Torque with test oil.....               | 19.8 |
|   | Relative efficiency of test oil         |      |

$$\frac{19.3}{19.8} \times 100 = 97.4\%$$

10 It might be added that the cutting oils are

|                                                                                                                                                                                                                                                                                                                                                                                                                                                                                                                                                                                                                                                                                                                                                                                          |
|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| applied to the taps by means of a circulation system.                                                                                                                                                                                                                                                                                                                                                                                                                                                                                                                                                                                                                                                                                                                                    |
| 40 OSTER THREADING TEST                                                                                                                                                                                                                                                                                                                                                                                                                                                                                                                                                                                                                                                                                                                                                                  |
| 45 The threading test is conducted on an Oster pipe threading machine by threading four, 4" pieces of SAE 1020 steel pipe. During these operations the power consumption is graphically recorded on a wattmeter as each oil is evaluated. At the end of the test the average net power required to thread the four nipples is calculated. In this manner, the power measurement is made on a standard reference oil and then the operation is repeated on the unknown oil. The threading efficiency of the unknown oil is then calculated by arbitrarily assigning an efficiency of 100 per cent to the reference oil and calculating the comparative efficiency of the unknown on a power requirement basis. The mathematics used are similar to those illustrated in the tapping test. |
| 50                                                                                                                                                                                                                                                                                                                                                                                                                                                                                                                                                                                                                                                                                                                                                                                       |
| 55                                                                                                                                                                                                                                                                                                                                                                                                                                                                                                                                                                                                                                                                                                                                                                                       |
| 60 DRILL LIFE TEST                                                                                                                                                                                                                                                                                                                                                                                                                                                                                                                                                                                                                                                                                                                                                                       |
| 65 The drill life test is determined by using ten drills uniformly ground to specified angles, three of which are placed in the chucks of a triple spindle head of the drill press at the start of the test. Holes are then drilled through flats of SAE 3140 steel until drill failure occurs. This is evidenced by excessive noise, tool burning and deterioration of the cutting edges. The failed drill is replaced with a newly ground one and the test is continued until all ten drills fail. The drill life with any oil is the average of the number of holes obtained per drill. During the test a continuous flow of cutting oil is supplied to each drill.                                                                                                                   |
| 70                                                                                                                                                                                                                                                                                                                                                                                                                                                                                                                                                                                                                                                                                                                                                                                       |
| 75 The results of the foregoing tests are tabulated in Table I.                                                                                                                                                                                                                                                                                                                                                                                                                                                                                                                                                                                                                                                                                                                          |

5  
Table I

| Additive                                           | Tapping Efficiency Per Cent | (Oster) Threading Efficiency Per Cent | Drill Life Number of Holes |
|----------------------------------------------------|-----------------------------|---------------------------------------|----------------------------|
| None <sup>1</sup>                                  | 90                          | 90                                    | 51                         |
| None <sup>2</sup>                                  | 80                          | 80                                    | -----                      |
| HOH                                                | 110                         | 102                                   | 79                         |
| HOH                                                | 111                         | 103                                   | -----                      |
| MGO                                                | 100                         | 100                                   | 64                         |
| DGO                                                | 100                         | 100                                   | 59                         |
| Commercial Hydro-abietal Alcohol <sup>3</sup>      | 106                         | 99                                    | 97                         |
| Commercial Hydro-abietal Alcohol <sup>4</sup> (5%) | 121                         | 101                                   | -----                      |

<sup>1</sup> Compound oil having mineral oil base and containing 0.9 per cent active sulfur.

<sup>2</sup> Compound oil having mineral oil base and containing at least 0.8 per cent non-corrosive sulfur and at least 0.75 per cent chlorine.

<sup>3</sup> Additive HOH is an ester of an hydroxy aliphatic dicarboxylic acid in which one carboxyl group is esterified by commercial hydro-abietyl alcohol and the other carboxyl group is esterified by a high molecular weight aliphatic alcohol.

<sup>4</sup> Additive MGO is an ester of a low molecular weight dihydric alcohol esterified with a high molecular weight aliphatic monocarboxylic acid and then esterified with a low molecular weight aliphatic dicarboxylic acid.

<sup>5</sup> Additive DGO is an ester of an hydroxy aliphatic dicarboxylic acid in which both carboxyl groups have been esterified by a high molecular weight aliphatic alcohol.

It will be noted that the most readily discerned difference is in the number of holes which can be drilled before a drill must be retired. The base oil containing 0.9% active sulfur permitted the drilling of 51 holes before the drill was retired. One ester type additive (DGO) when added to the base oil increased the drill life about 16 per cent; a second ester type additive (MGO) increased drill life about 26 per cent; the third ester type additive (HOH) increased drill life about 55 per cent. However, 1 per cent commercial hydroabietyl alcohol increased drill life 90 per cent or almost doubled the life of the drill.

Satisfactory results can be obtained when employing other base oils as for example, mineral oil of lubricating grade admixed with a moderately sulfurized mineral oil containing about 0.9 per cent active sulfur and a chlorinated paraffine base containing about 42 per cent chlorine. The commercially available hydroabietyl alcohol can be mixed with the aforementioned components and other additives such as stain inhibitors, antioxidants, etc. to provide a composite oil having a composition coming within the ranges set forth hereinafter:

|                                                                                       | Broad Formula | Preferred Formula |
|---------------------------------------------------------------------------------------|---------------|-------------------|
| <b>Formula A:</b>                                                                     |               |                   |
| Moderately sulfurized Mineral oil containing about 0.9% active sulfur; per cent       | 0-99          | 30-99             |
| Chlorinated base containing about 42% chlorine; per cent                              | 0-15          | 0-7               |
| Mineral oil 50-500°@100° F. SUV; per cent                                             | 0-99          | 0-62              |
| Commercial Hydroabietyl Alcohol; per cent                                             | 0.1-10        | 0.25-2            |
| <b>Formula B:</b>                                                                     |               |                   |
| Sulfurized-chlorinated fatty oil containing about 5% sulfur and about 5% Cl; per cent | 0.25-15       | 0.5-4.0           |
| Mineral oil, 50-500°@100° F. SUV; per cent                                            | 78-99         | 95-99             |
| Stain Inhibitor; per cent                                                             | 0-2           | 0.1-0.5           |
| Commercial Hydroabietyl Alcohol; per cent                                             | 0.1-5         | 0.25-0.5          |

In view of the foregoing it is manifest that improved results can be obtained in gear lubricants, cutting oils and the like by incorporating commercial hydroabietyl alcohol in the compound oil as an oiliness additive. Those skilled in the art will understand that other additives such as stain inhibitors, antioxidants and the like can also be incorporated in the usual amounts.

## 6

While the Tapping, Threading and "Drill Life" tests indicate that esters having both carboxyl groups of a hydroxy aliphatic polycarboxylic acid esterified with radicals from hydroabietyl alcohol mixture are all more effective than similar esters of aliphatic alcohols there is an advantage to the use of either mixed esters or mixtures of esters. This advantage results from the viscosity of the various esters. As is manifest after a consideration of the following tabulation of viscosities of various esters, di-hydroabietyl malate, for example, is far more viscous than the mixed esters. The high viscosity of the di-hydroabietyl esters makes it desirable to reduce the viscosity without sacrificing a disproportionate amount of the effectiveness of the hydroabietyl esters. As will be appreciated by study of the following tabulation this can be done by using mixed esters.

| Ester                              | Tapping Efficiency, Per Cent | Oster Threading Efficiency, Per Cent | Viscosity at 130° F. | SUV (sec) at 210° F. |
|------------------------------------|------------------------------|--------------------------------------|----------------------|----------------------|
| Di-hydroabietyl malate             | 101                          | 101                                  | -----                | 2,641                |
| Hydroabietyl oleyl malate          | 110                          | 102                                  | 730                  | 104                  |
| Hydroabietyl-1-2-ethylhexyl malate | 102                          | 100                                  | 1,668                | 134                  |

Consequently, for ease of manufacture and incorporation in oil blends it is preferred to employ a mixed ester of an alpha-hydroxy polycarboxylic acid derived from 50 mole per cent of hydroabietyl alcohol and 50 mole per cent oleyl alcohol, i. e., from the reaction of 1 mole of hydroabietyl alcohol, 1 mole of oleyl alcohol and 1 mole of polycarboxylic acid. Fluidity of the product can be obtained by employing mixed esters of alpha-hydroxy polycarboxylic aliphatic acids in which from 50 mole per cent to 99 mole per cent hydroabietyl radical and from 1 to 50 mole per cent of an alkyl radical are present in the carbalkoxy groups. The alkyl groups are those derived from monohydric saturated or unsaturated alcohols having from one through 18 carbon atoms and includes oleyl alcohol.

Mixed esters containing 75 mole per cent hydroabietyl, 25 mole per cent oleyl ester may be made in any of the following or other suitable procedures.

A. Hydroabietyl alcohol (about 1.5 moles) oleyl alcohol (about 0.5 mole) and alpha-hydroxy aliphatic polycarboxylic acid (about 1.0 mole) are reacted as described hereinbefore.

B. About 75 mole parts of di-hydroabietyl ester of an alpha-hydroxy aliphatic polycarboxylic acid and about 25 mole parts of di-oleyl ester of an alpha-hydroxy aliphatic polycarboxylic acid are heated together until ester exchange has occurred.

C. Equal parts of 85 mole per cent hydroabietyl-15 mole per cent oleyl ester of an alpha-hydroxy aliphatic polycarboxylic acid and of 65 mole per cent hydroabietyl-35 mole per cent oleyl ester of an alpha-hydroxy aliphatic polycarboxylic acid are heated together until ester exchange has occurred. Thus, for example, the esters may be the malates.

It is to be noted that while the neutral esters are satisfactory for use in cutting oils it is preferred to use esters which are a mixture of neutral and partial esters for anti-rust agents. Therefore it is preferred to use esters having a neutralization number of zero to 30 in cutting

oils but esters having a minimum neutralization number of 10 in anti-rust oils, such as turbine oils.

In the copending application for United States Letters Patent Serial No. 86,382, filed April 8, 1949, now Patent No. 2,564,634, patented August 14, 1951, in the names of Leslie C. Beard and Ralph V. White, there is a disclosure of the improved results accruing from the use of an ester of a hydroxy aliphatic polycarboxylic acid in which at least one carboxyl group of said acid is esterified by hydroabietyl alcohol in turbine oils, cutting oils and the like. It has been discovered that the improved results obtained by incorporating an ester of the class defined hereinbefore in mineral oil compositions can be still further improved by incorporating hydroabietyl alcohol in addition to the aforesaid ester. This will become apparent from the data presented in Table II for cutting oil compositions.

Table II

| Additive          | Percent Weight | Tapping Efficiency Percent | Oster Threading Efficiency Percent | Drill Life Number of Holes |
|-------------------|----------------|----------------------------|------------------------------------|----------------------------|
| None <sup>1</sup> |                | 90                         | 90                                 | 51                         |
| HOH               | 1              | 110                        | 102                                | 79                         |
| HOH               | 0.75           | 114                        | 98                                 | 87                         |
| Hal               | 0.25           |                            |                                    |                            |
| HHO               | 1              | 102                        | 101                                |                            |
| HHO               | 0.75           | 107                        | 101                                | 101                        |
| Hal               | 0.25           |                            |                                    |                            |
| HEO               | 1              | 102                        | 100                                |                            |
| HEO               | 0.75           | 107                        | 101                                | 82                         |
| Hal               | 0.25           |                            |                                    |                            |
| MGO               | 1              | 100                        | 100                                | 64                         |

<sup>1</sup> Compound oil having mineral oil base and containing 0.9 per cent active sulfur.

Additive HOH is an ester of a hydroxy aliphatic dicarboxylic acid in which one carboxyl group is esterified by commercial hydroabietyl alcohol and the other carboxyl group is esterified by a high molecular weight aliphatic alcohol.

Additive HHO is an ester of a hydroxy aliphatic dicarboxylic acid in which both carboxyl groups are esterified by commercial hydroabietyl alcohol.

Additive HEO is an ester of a hydroxy aliphatic dicarboxylic acid in which one carboxyl group is esterified by commercial hydroabietyl alcohol and the other carboxyl group is esterified by a mono-hydro aliphatic alcohol having eight carbon atoms in the molecule.

Additive Hal is commercial hydroabietyl alcohol.

It will be noted that when about 25% of the hydroabietyl ester additive is replaced by hydroabietyl alcohol per se the properties of the blend are superior to those of the blend of base oil and ester. Thus, for example, the drill life, when the base oil is used without ester or hydroabietyl alcohol, is only 51 holes. When 1 weight per cent of additive HOH is incorporated in the base oil the drill life is increased 55%, i. e., from 51 to 79 holes. When 0.75% HOH and 0.25% hydroabietyl alcohol are incorporated in the base oil the drill life is increased 71%. Thus, it is evident that improved results can be obtained not only when hydroabietyl alcohol is the sole additive for this purpose but also when the hydroabietyl alcohol is only 25% of the total additive of this class present in the oil. Therefore, it is within the scope of the present invention to use 0.1 to 5% of hydroabietyl alcohol or a mixture of hydroabietyl alcohol and an ester of an hydroxy aliphatic polycarboxylic acid in which at least one carboxyl group is esterified by hydroabietyl alcohol, said ester being present in an amount not greater than 4 times the concentration of the hydroabietyl alcohol and the minimum concentration of hydroabietyl alcohol per se being 0.20 weight per cent.

As those skilled in the art will understand other additives such as stain inhibitors, anti-oxidants and the like can also be incorporated in the usual

amounts in addition to the additives specifically defined hereinbefore.

We claim:

5 1. A compound oil consisting essentially of a mineral oil base of lubricating grade containing about 0.9 per cent active sulfur and commercial hydroabietyl alcohol in amount of 0.1 to about 10% effective to increase drill life.

10 2. A compound oil consisting essentially of a mineral oil base of lubricating grade, containing at least 0.8 per cent non-corrosive sulfur, at least 0.75 per cent chlorine and commercial hydroabietyl alcohol in amount of 0.1 to about 10% effective to increase drill life.

15 3. A compound oil consisting essentially of

|                                                 | Per cent |
|-------------------------------------------------|----------|
| Mineral oil containing about 0.9% active sulfur | 30-99    |

|                                                |     |
|------------------------------------------------|-----|
| Chlorinated base containing about 42% chlorine | 0-7 |
|------------------------------------------------|-----|

|                                                |      |
|------------------------------------------------|------|
| Mineral oil, 50-500 seconds S. U. V. @ 100° F. | 0-62 |
|------------------------------------------------|------|

|                                 |        |
|---------------------------------|--------|
| Commercial hydroabietyl alcohol | 0.25-2 |
|---------------------------------|--------|

25 4. A compound oil consisting essentially of

|                                                                                   | Per cent |
|-----------------------------------------------------------------------------------|----------|
| Sulfurized-chlorinated fatty oil containing about 5% sulfur and about 5% chlorine | 0.25-15  |

|                                                   |       |
|---------------------------------------------------|-------|
| 30 Mineral oil, 50-500 seconds S. U. V. @ 100° F. | 78-99 |
|---------------------------------------------------|-------|

|                 |     |
|-----------------|-----|
| Stain inhibitor | 0-2 |
|-----------------|-----|

|                                 |       |
|---------------------------------|-------|
| Commercial hydroabietyl alcohol | 0.1-5 |
|---------------------------------|-------|

35 5. A compound oil consisting essentially of

|                                                                                   | Per cent |
|-----------------------------------------------------------------------------------|----------|
| Sulfurized-chlorinated fatty oil containing about 5% sulfur and about 5% chlorine | 0.5-4.0  |

|                                                   |       |
|---------------------------------------------------|-------|
| 40 Mineral oil, 50-500 seconds S. U. V. @ 100° F. | 95-99 |
|---------------------------------------------------|-------|

|                 |         |
|-----------------|---------|
| Stain inhibitor | 0.1-0.5 |
|-----------------|---------|

|                                 |          |
|---------------------------------|----------|
| Commercial hydroabietyl alcohol | 0.25-0.5 |
|---------------------------------|----------|

6. A compound oil consisting essentially of a

45 major proportion of a lubricating fraction of mineral oil containing about 0.9 per cent active sulfur and an amount of 0.1 to about 10% effective to increase drill life of a mixture of commercial hydroabietyl alcohol and esters of malic acid, said mixture of hydroabietyl alcohol and esters consisting essentially of at least 0.2 weight

50 per cent hydroabietyl alcohol and the balance an ester product of malic acid in which about 50-100 mol per cent of the radicals attached to

55 the carbonyl carbon atoms through oxygen is radicals of hydroabietyl alcohol and the balance is a radical of monohydric aliphatic alcohol having 8-20 carbon atoms, the concentration of said esters in said mixture being not greater than

60 four times the concentration of said commercial hydroabietyl alcohol and said esters having a minimum neutralization number of 10.

7. A compound oil consisting essentially of a major proportion of a lubricating fraction of

65 mineral oil containing about 0.9 per cent active sulfur and an amount of 0.1 to about 10% effective to increase drill life of a mixture of commercial hydroabietyl alcohol and esters of malic acid, said mixture consisting essentially of at

70 least 0.2 weight per cent commercial hydroabietyl alcohol and the balance an ester product of malic acid in which about 50-100 mol per cent of the radicals attached to the carbonyl carbon atoms through oxygen is radicals of commercial hydroabietyl alcohol and the balance is a radical of

monohydric aliphatic alcohol having 8-20 carbon atoms, said ester being present in said mixture of commercial hydroabietyl alcohol and ester in a concentration not greater than four times the concentration of said commercial hydroabietyl alcohol, said ester having a neutralization number of zero to 30 and the concentration of said commercial hydroabietyl alcohol in said compound oil being at least 0.20 weight per cent.

8. A compound oil consisting essentially of a mixture of hydroabietyl alcohol and an ester 0.1% - 5%, chlorinated base containing about 42% chlorine 0-15%, and the balance not to exceed 99% of at least one oleaginous vehicle selected from the group consisting of mineral oil containing about 0.9% active sulfur and mineral oil of 50-500 seconds S. U. V. @ 100° F., said mixture of hydroabietyl alcohol and ester consisting essentially of at least 0.2 weight per cent hydroabietyl alcohol and the balance an ester product of malic acid in which about 50-100 mol per cent of the radicals attached to the carbonyl carbon atoms through oxygen is radicals of hydroabietyl alcohol and the balance is a radical of monohydric aliphatic alcohol having 8-20 carbon atoms, said ester being in a concentration not greater than four times the concentration of said hydroabietyl alcohol, and said ester having a neutralization number of zero to 30.

9. A compound oil as described and set forth in claim 8 wherein the mixture of hydroabietyl alcohol and an ester consists essentially of a mixture of commercial hydroabietyl alcohol and esters containing 75 mole per cent of an ester of malic acid and an alcohol derived from commercial hydroabietyl alcohol and 25 mole per cent of an ester of malic acid and oleyl alcohol.

10. A compound oil as described and set forth in claim 8 wherein the ester consists essentially of 75 mole per cent of an ester of malic acid and an alcohol derived from commercial hydroabietyl alcohol and 25 mole per cent of an ester of said malic acid and oleyl alcohol.

11. A compound oil as described and set forth

in claim 8 wherein the ester consists essentially of mixed esters of malic acid in which 50 to 99 mole per cent of the carbalkoxy groups is derived from commercial hydroabietyl alcohol and 1 to 50 mole per cent of the carbalkoxy groups is an alkyl group having 1 to 18 carbon atoms.

12. A compound oil as described and set forth in claim 8 wherein the ester consists essentially of mixed esters of malic acid in which 50-99 mole percent of the carbalkoxy group is derived from commercial hydroabietyl alcohol and, 1 to 50 mole per cent of the carbalkoxy groups is derived from a monohydric aliphatic alcohol having 1 through 18 carbon atoms.

13. A compound oil consisting essentially of commercial hydroabietyl alcohol 0.1 to 10%, chlorinated base containing about 42% chlorine 0-15% and the balance not to exceed 99% of at least one oleaginous vehicle selected from the group consisting of mineral oil of 50-500 seconds S. U. V. @ 100° F. and mineral oil containing about 0.9% active sulfur.

SAMUEL MANILYCH.  
LEE L. LAMBERT.

#### REFERENCES CITED

The following references are of record in the file of this patent:

#### UNITED STATES PATENTS

| Number    | Name         | Date           |
|-----------|--------------|----------------|
| 2,021,100 | Henke        | Nov. 12, 1935  |
| 2,094,127 | Lazier       | Sept. 28, 1937 |
| 2,142,989 | Barrett      | Jan. 10, 1939  |
| 2,268,608 | McNulty      | Jan. 6, 1942   |
| 2,274,617 | Remy         | Feb. 24, 1942  |
| 2,384,595 | Blair        | Sept. 11, 1945 |
| 2,430,058 | Kluber       | Nov. 4, 1947   |
| 2,443,578 | Fuller       | June 15, 1948  |
| 2,564,638 | Beard et al. | Aug. 14, 1951  |

#### OTHER REFERENCES

"New Products and Materials" in Chemical Engineering, Jan. 1948, p. 173.

Patent No. 2,591,570

Certificate of Correction

April 1, 1952

SAMUEL MANILYCH ET AL.

It is hereby certified that error appears in the printed specification of the above numbered patent requiring correction as follows:

Column 1, line 35, for "Saponification" read *Saponification*; column 3, line 39, for "alchols" read *alcohols*; column 4, line 8, for "109" read *100*; column 9, line 30, for "an" read *and*; column 10, line 12, for "mile" read *mole*; and that the said Letters Patent should be read as corrected above, so that the same may conform to the record of the case in the Patent Office.

Signed and sealed this 25th day of November, A. D. 1952.

[SEAL]

THOMAS F. MURPHY,  
*Assistant Commissioner of Patents.*